

Patented Apr. 1, 1924.

1,489,118

# UNITED STATES PATENT OFFICE.

ANTHONY J. FREITAS, OF ERIE, PENNSYLVANIA.

## METHOD OF TREATING STEEL.

No Drawing.

Application filed January 12, 1921. Serial No. 436,817.

To all whom it may concern:

Be it known that I, ANTHONY J. FREITAS, a citizen of the United States, residing at Erie, in the county of Erie and State of Pennsylvania, have invented new and useful Improvements in Methods of Treating Steel, of which the following is a specification.

The invention is designed to improve the quality of steel. In accomplishing this purpose I treat the steel while in the molten state with a compound containing preferably potassium prussiate yellow, fuller's-earth and charcoal. The compound is preferably made up of forty parts of potassium prussiate yellow, two parts fuller's-earth, and six parts charcoal, and in the treatment of most steels the application or introduction of about two and a quarter pounds of this compound to each ton of steel gives the best results.

This material may be introduced to the steel in the furnace, in the crucible or in the ladle, preferably in the ladle because the melting losses are thus avoided.

The addition of the material to the molten steel results in the momentary increase in temperature of the steel and changes its quality without materially changing its chemical analysis.

It apparently increases all the ordinary physical characteristics, such as tensile strain, elasticity, elongation and reduction of area, both in annealed and cast forgings and in the quenched and drawn steel. It also seems to vary the transformation point so that the steel may be better annealed and thus adding to its availability for forging and machining. It also seems to permit of a decrease in such ingredients as manganese and silicon without deterioration of the quality of the steel. The addition of the material seems to change the fiber structure so as to avoid to a large extent the cracking during quenching and increases the ductility and also varies its density so as to decrease

the shrinkage in casting. The steel also seems to stand a higher temperature and the quantity of scale is reduced.

The invention is particularly desirable in forming cast steel and in doing this the practice is to add the material as the steel is delivered from the furnace to the ladle.

What I claim as new is:

1. The method of treating steel which consists in adding to the steel while in a molten state potassium prussiate, a material having aluminum as a base and carbon.

2. The method of treating steel which consists in adding to the steel while in a molten state potassium prussiate forty parts, a material having aluminum as a base two parts, and carbon six parts.

3. The method of treating steel which consists in adding to the steel while in a molten state potassium prussiate forty parts, fuller's-earth two parts, and charcoal six parts.

4. The method of treating steel which consists in adding to the steel while in a molten state potassium prussiate forty parts, a material having aluminum as a base two parts, and carbon six parts in quantities amounting to two and a quarter pounds to the ton of steel.

5. The method of treating steel which consists in adding to the steel while in a molten state potassium prussiate forty parts, fuller's-earth two parts, and charcoal six parts, in quantities amounting to two and a quarter pounds to the ton of steel.

6. A compound for treating steel comprising forty parts of potassium prussiate yellow, two parts of material having aluminum as a base, and six parts of carbon.

7. The method of forming cast steel which consists in treating the molten metal with a compound of potassium prussiate, fuller's-earth and carbon.

In testimony whereof I have hereunto set my hand.

ANTHONY J. FREITAS.